

## UNITED STATES PATENT OFFICE

2,165,265

## PROCESS OF IMPARTING HYDROPHOBIC PROPERTIES TO CELLULOSE FIBERS

Franz Emil Hubert, Dessau-Ziebigk, Erwin Heisemberg, Leipzig, and Adolf Steindorff and Ludwig Orthner, Frankfort-on-the-Main, Germany, assignors to I. G. Farbenindustrie Aktiengesellschaft, Frankfort-on-the-Main, Germany

No Drawing. Application May 21, 1936, Serial No. 81,122. In Germany May 11, 1935

5 Claims. (Cl. 91—70)

The present invention relates to a process of imparting hydrophobic properties to cellulose fibers.

It is known that fibers of cellulose or hydrated cellulose, such as cotton, artificial silk or staple fiber are extraordinarily hydrophil, that is to say they are very quickly wetted when in contact with water. This property is a great disadvantage for many of the applications of this material.

10 This invention consists in a process for making cellulose fibers hydrophobe by applying to the fibers or incorporating with them a compound which contains at least one aliphatic or cycloaliphatic residue having at least 4 carbon atoms

15 and capable of reacting with aldehyde and exposing the fibers thus treated simultaneously or subsequently to the action of an aliphatic aldehyde or dialdehyde, for instance, formaldehyde or glyoxal.

20 Suitable aliphatic compounds are, for example, fatty amines and fatty acid amides such as dodecylamine, hexadecylamine, octadecenylamine, abietic acid amide, lauric acid amide, stearoyl-methylamide, stearoyl-butylamide, stearoyloctadecylamide; further compounds of the character of alkyl-substituted ureas having the general formula:



25 wherein R stands for a radical selected from the group consisting of aliphatic and cycloaliphatic radicals containing at least 4 carbon atoms, X stands for a member selected from the group consisting of O, NH, N. alkyl, and R<sub>1</sub> stands for a member of the group consisting of hydrogen and aliphatic hydrocarbon radicals, such as mono-isobutyl urea, monododecyl urea, mono-octadecyl urea, stearoyl urea; further fatty acid imino ethers or amidines. There also come into consideration compounds containing hydroxyl groups, such as, for instance, dodecylphenol, di-isohexyl-phenol. Instead of the products named 30 above there may also be used with advantage their products of reaction with aliphatic aldehydes, for example, their methylol compounds. If these latter are used the separate after-treatment with formaldehyde can be omitted in many 35 cases, a simple after-heating operation sufficing.

40 The process may be conducted, for example, as follows: the cellulose fibers are first saturated with a solution of the aliphatic compound in an organic solvent, for instance, pyridine, or acetone or in an aqueous emulsion of the aliphatic com-

pounds. They are then dried and exposed to the action of, for instance, formaldehyde, the concentration of which, when it is used in the form of a solution, must not be more than 5%. The formaldehyde may be added to the impregnating solution so that a subsequent treatment with formaldehyde becomes unnecessary; however, care must likewise be taken that the concentration of the aldehyde, for instance, of the formaldehyde, in the treating solution is not more than 5%. In this case the fiber needs only subsequent heating to ensure sufficient reaction of the formaldehyde with the impregnating compound and the fiber.

5 In many cases it is useful to conduct the subsequent heating in an acid medium. For this purpose there may be added, for example, to the aqueous emulsion, acetic acid, lactic acid or agents of acid reaction such as sodium bisulfite.

10 Fibers treated in this manner are characterized by a particularly high stability towards water and even hot soap solution. For example, such material can be subjected to the usual fulling treatment, that is to say heating for 1/2 hour in a solution of 50 grams of soap and 5 grams of sodium carbonate per liter at 50° C. without loss of the property of repellent water. By suitable combination of the parent material and working conditions an effect can be obtained 15 which is not notably diminished by several washings with boiling soap solution.

20 Another process of rendering cellulose fibers water-repellent consists in treating the fibers with solutions or dispersions of the aldehyde condensation products. As a catalyst an acid 25 substance is suitably added to the solutions or dispersions. The fibers may also be pretreated with an acid substance. The said aldehyde condensation products may also be added directly to the spinning solutions from which the artificial 30 cellulose threads are prepared. The fibers which are prepared from solutions containing such an addition may, if required, be treated subsequently with an aldehyde.

35 The following examples serve to illustrate the invention, but they are not intended to limit it thereto; the parts are by weight:

40 1. Unsoaped dry viscose silk is immersed for 5 minutes in 5 times its weight of a pyridine solution containing 5-10 per cent. of octadecyl- 45 heptadecyl urea of the formula:



55

- The silk is then drained, dried, immersed for 5 minutes in aqueous formaldehyde solution of 30 per cent. strength, centrifuged, dried and heated for 16 hours at 100° C. Instead of this treatment with formaldehyde the fibrous material may be suspended for 1/2 hour in a chamber charged with formaldehyde vapor at 110° C. Instead of octadecyl-heptadecyl urea another of the substances specified above may be used.
10. 2. Unsoaped dry viscose silk is immersed for 5 minutes in 10 times its weight of an aqueous emulsion containing 2 per cent. of stearin-amide, 0.2 per cent. of an emulsifying agent, obtainable by the reaction of ethylene-oxide with octadecenyl-alcohol, and 0.3 percent. of formaldehyde.
15. 3. Unsoaped, dry viscose silk is immersed for 5 minutes in 5 times its weight of a solution of 5-10 per cent. strength of methylol-stearin-amide in pyridine. The goods are centrifuged, dried and heated for 6 hours at 110° C. A subsequent washing is not necessary.
20. 4. The operation is conducted as described in Example 2 but 7 per cent. of lactic acid is added to the emulsion. By this addition of acid the stability of the water repelling preparation is strongly increased, particularly towards treatment with boiling dilute acid.
25. 5. 10 parts of monostearylamino-cyanuric diamide are dissolved by warming 50 parts of a 10% lactic acid solution until the mass is homogeneous. The whole is made up with water to 2000 parts and while stirring, 40 parts of 30 formaldehyde of 40 per cent. strength are added. A viscose artificial silk fabric is impregnated with this solution, squeezed, dried at moderate temperature and thereupon heated for 15 minutes at 155° C. to 160° C. The tissue thus treated is very water-repellent even after the usual washing with soap.
35. A similar good effect is also obtained by causing other amino derivatives of the 1,3,5-triazine, containing an alkyl radical with at least 4 carbon atoms, to act upon the cellulose fibers and treating them, either simultaneously or subsequently, with aliphatic aldehydes. For example the 1,3,5-triazine of the formula:
- 40.
- 30.
- 35.
- 40.
- 45.
- 50.
- 55.
- 60.
- 65.
- 70.
- 75.



of 40° C. to 50° C. The tissue is then heated for 5-10 minutes at a temperature of 130° C. to 140° C.

8. Undyed or dyed viscose artificial silk is treated with a solution which contains per liter of water 5 grams of lactic acid or glycolic acid, and is then dried. This pretreated material is treated for 10 minutes at 60° C. to 70° C. with a solution of a condensation product, obtainable from montanic acid amide and aqueous formaldehyde, in carbon tetrachloride. The material is squeezed, dried and heated for some minutes at a temperature of 140° C. There is thus obtained a hydrophobe tissue having a very good water-repellent effect.

9. 4 parts of viscose artificial silk are impregnated with 100 parts by volume of a 1 per cent. solution of dodecylvinylether in dioxane, squeezed and dried. The silk is then loosened and heated for 2 hours at 110° C. under reduced pressure in an atmosphere of glacial acetic acid and formaldehyde. Thereupon it is washed while cold, hydro-extracted and dried. The viscose silk is very water-repellent and resistant to boiling.

10. Dyed viscose artificial silk fabric is immersed in a 2 per cent. solution of carbamic acid-octadecyl ester having the formula:



in methylene chloride for about 10 minutes, then squeezed and after evaporation of the solvent the material is conducted through a bath which contains 5 per cent. of formaldehyde and 0.5 per cent. of lactic acid. The material is then dried in a tentering frame for about half-an-hour at 105° C. to 110° C. Even after washing with soap the material is water-repellent and impermeable to water.

Instead of viscose artificial silk, cellulose fibers of all kinds, for instance, copper artificial silk, artificial spinning fibers, cotton, also mixtures of wool and cellulose fibers as well as fabrics made from the said fibers and mixtures of fibers may be used. In some cases a preliminary cleansing or desizing of the fibers or fabric is advisable.

We claim:

1. The process of imparting hydrophobic properties to cellulose fibers by impregnating the fibers in a bath which contains compounds of the general formula:



wherein R stands for a radical selected from the group consisting of aliphatic and cycloaliphatic radicals containing at least 4 carbon atoms, X stands for a member selected from the group consisting of O, NH, N.alkyl and R<sub>1</sub> stands for a member of the group consisting of hydrogen and, aliphatic hydrocarbon radicals, and at most 5 per cent. of aldehyde, and heating them after the impregnation.

2. The process of imparting hydrophobic properties to cellulose fibers by impregnating the fibers in a bath which contains compounds of the general formula:



wherein R stands for a radical selected from the group consisting of aliphatic and cycloaliphatic radicals containing at least 4 carbon atoms, X stands for a member selected from the

group consisting of O, NH, N.alkyl and R<sub>1</sub> stands for a member of the group consisting of hydrogen and, aliphatic hydrocarbon radicals, at most 5 per cent. of aldehyde and an agent of acid action, 5 and heating them after the impregnation.

3. The process of imparting hydrophobic properties to cellulose fibers by incorporating with them a compound of the general formula:

10



wherein R stands for a radical selected from the group consisting of aliphatic and cycloaliphatic radicals, containing at least 4 carbon atoms, X 15 stands for a radical selected from the group consisting of O, NH, N.alkyl and R<sub>1</sub> stands for a member of the group consisting of hydrogen and aliphatic hydrocarbon radicals, treating the fibers 20 with aliphatic aldehydes and subsequently heating them.

4. The process of imparting hydrophobic properties to cellulose fibers by impregnating the fibers with a condensation product from an aldehyde 25 and a compound of the general formula:



wherein R stands for a radical selected from the group consisting of aliphatic and cycloaliphatic radicals containing at least 4 carbon atoms, X 5 stands for a radical selected from the group consisting of O, NH, N.alkyl and R<sub>1</sub> stands for a member of the group consisting of hydrogen and aliphatic hydrocarbon radicals, and heating them after the impregnation.

5. The process of imparting hydrophobic properties to cellulose fibers by impregnating the 10 fibers with a condensation product from an aldehyde and a compound of the general formula:



15

wherein R stands for a radical selected from the group consisting of aliphatic and cycloaliphatic radicals containing at least 4 carbon atoms, X 20 stands for a radical selected from the group consisting of O, NH, N.alkyl and R<sub>1</sub> stands for a member of the group consisting of hydrogen and aliphatic hydrocarbon radicals, in the presence of an agent of acid action, and heating them after 25 the impregnation.

FRANZ EMIL HUBERT.  
ERWIN HEISENBERG.  
ADOLF STEINDORFF.  
LUDWIG ORTHNER.